

## [54] HIGHLY-HANDLEABLE PITCH-BASED FIBERS

[75] Inventor: David A. Schulz, Fairview Park, Ohio

[73] Assignee: Union Carbide Corporation, New York, N.Y.

[21] Appl. No.: 793,512

[22] Filed: May 4, 1977

## Related U.S. Application Data

[60] Continuation of Ser. No. 657,208, Feb. 11, 1976, abandoned, which is a division of Ser. No. 562,777, Mar. 27, 1975, Pat. No. 4,014,725.

[51] Int. Cl.<sup>2</sup> ..... B32B 9/00; B29C 25/00; D02G 3/00

[52] U.S. Cl. ..... 428/367; 264/29.2; 264/176 F; 264/344; 423/447.1; 423/447.6; 428/401

[58] Field of Search ..... 428/367, 401; 423/447.6, 447.1; 264/29, 344, 176 F, 29.6; 156/148

## [56] References Cited

## U.S. PATENT DOCUMENTS

|           |         |                        |           |
|-----------|---------|------------------------|-----------|
| 3,541,582 | 11/1970 | Johnson et al. ....    | 23/209.1  |
| 3,595,946 | 7/1971  | Joo et al. ....        | 264/82 X  |
| 3,629,379 | 12/1971 | Otani ....             | 423/447.5 |
| 3,702,054 | 11/1972 | Araki et al. ....      | 423/447.6 |
| 3,716,607 | 2/1973  | Otani et al. ....      | 264/29.6  |
| 3,787,541 | 1/1974  | Grindstaff et al. .... | 423/447.1 |

|           |         |                   |           |
|-----------|---------|-------------------|-----------|
| 3,919,387 | 11/1975 | Singer .....      | 264/344   |
| 3,943,213 | 3/1976  | Whittaker .....   | 264/29    |
| 3,974,264 | 8/1976  | McHenry .....     | 423/447.6 |
| 4,005,183 | 1/1977  | Singer .....      | 423/447.2 |
| 4,016,247 | 4/1977  | Otani et al. .... | 423/447.6 |
| 4,032,430 | 6/1977  | Lewis .....       | 423/447.1 |

## FOREIGN PATENT DOCUMENTS

1071400 9/1964 United Kingdom ..... 423/447.6

## OTHER PUBLICATIONS

Otani, S., "On the Carbon Fiber from the Molten Pyrolysis Products", Carbon, vol. 3, pp. 31-38, 1965.

Bacon, R., Pallozzi, A. A., Slosarik, S. E., "Carbon Fiber", Modern Plastics, pp. 608-610, 1966.

*Primary Examiner*—Lorraine T. Kendall  
*Attorney, Agent, or Firm*—John S. Piscitello

## [57]

## ABSTRACT

Fibers having a high degree of flexibility and handleability are produced by oxidizing fibers spun from a carbonaceous pitch which has been transformed, in part, to a liquid crystal or so-called "mesophase" state to an oxygen content of from 17 per cent by weight to 30 per cent by weight. Because of their strength and handleability, these highly-oxidized fibers can be easily processed at high speeds by means of conventional yarn-transport systems, and readily woven or knit into cloth. Such cloth may then be heat treated to produce carbon or graphite cloth.

24 Claims, No Drawings

**HIGHLY-HANDLEABLE PITCH-BASED FIBERS**

This application is a continuation of our prior U.S. application Ser. No. 657,208, filing date Feb. 11, 1976, and now abandoned, which is a division of application Ser. No. 562,777, filing date Mar. 27, 1975, now U.S. Pat. No. 4,014,725.

**BACKGROUND OF THE INVENTION****1. Field of the Invention**

This invention relates to highly-oxidized pitch fibers having a high degree of flexibility and handleability which can be easily processed to produce carbon or graphite fibers, or woven or knit to produce a fabric which in turn may be heat treated to produce a carbon 15 or graphite cloth.

**2. Description of the Prior Art**

The production of carbon and graphite fibers from pitch is well known in the art. Such fibers are usually produced by spinning a fiber from the pitch, thermosetting the fiber so produced by heating the fiber in an oxygen-containing atmosphere for a time sufficient to render it infusible, and then heating the infusible fiber to a carbonizing or graphitizing temperature in an inert atmosphere. While the carbonized or graphitized fibers produced in this manner are characterized by high strength, the as-spun and oxidized fibers have a very low strength. For this reason, such fibers are difficult to work with and considerable care must be exercised in processing such fibers to carbon and graphite to avoid 30 breakage of the fibers.

Because of the low strength of the as-spun and oxidized fibers, it is customary to first carbonize or graphitize such fibers in order to improve their strength before attempting to weave or knit them into a cloth. However, while the carbonized and graphitized fibers have 35 high strength, they also are characterized by high modulus which makes them difficult to work with because of their brittleness.

**SUMMARY OF THE INVENTION**

In accordance with the present invention, it has now been discovered that the tensile strength and handleability of fibers spun from a carbonaceous pitch which has been transformed, in part, to a liquid crystal or so-called "mesophase" state can be significantly improved by oxidizing the fibers to an oxygen content of from 17 per cent by weight to 30 per cent by weight, preferably by from 18 per cent by weight to 22 per cent by weight.

While those skilled in the art initially sought to limit oxidation of pitch fibers to the minimum amount required to thermoset them in the belief that excessive oxidation would reduce the strength of the carbonized and graphitized fibers produced therefrom, it has now been discovered, quite surprisingly, that not only does oxidation to the high level stated above greatly increase the strength of the spun filament, but also, that it has no deleterious effect on the strength of the carbonized or graphitized fibers produced therefrom.

Because of their greater strength and handleability, the highly-oxidized fibers of the present invention are less subject to breakage and damage during subsequent thermal processing. This allows such fibers to be processed at high speeds by means of conventional yarn-transport systems where the fibers are subject to higher tensions and rougher treatment than the lower-oxidized fibers are capable of withstanding. Thus, such fibers can be rapidly transported through eyelets, over pulleys,

through furnaces, and wound at high speeds while the lower-oxidized fibers cannot. In addition, the high handleability of these fibers allows them to be utilized in textile-type processes, such as weaving or knitting, where demanding high-speed operations limit the use of the more fragile lower-oxidized fibers. The cloth produced from these processes may, of course, then be further processed to produce carbon or graphite cloth by further heat treatment, thereby eliminating the difficulty of weaving or knitting cloth from fibers which have been stiffened to a high modulus by such thermal processing.

**DESCRIPTION OF THE PREFERRED EMBODIMENTS**

While carbonaceous fibers can be spun from non-mesophase pitches, only mesophase pitches are employed in the present invention because of their ability to produce highly-oriented fibers which can be thermoset to produce a highly flexible, handleable fiber which can be further processed to produce high modulus, high strength carbon and graphite fibers. Mesophase pitches are pitches which have been transformed, in whole or in part, to a liquid crystal or so-called "mesophase" state. Such pitches by nature contain highly oriented molecules, and when these pitches are spun into fibers, the pitch molecules are preferentially aligned by the spinning process along the longitudinal axis of the fiber to produce a highly oriented fiber.

Mesophase pitches can be produced in accordance with known techniques by heating a natural or synthetic carbonaceous pitch having an aromatic base in an inert atmosphere at a temperature of above about 350° C. for a time sufficient to produce the desired quantity of mesophase. When such a pitch is heated in this manner under quiescent conditions, either at constant temperature or with gradually increasing temperature, small insoluble liquid spheres begin to appear in the pitch which gradually increase in size as heating is continued.

When examined by electron diffraction and polarized light techniques, these spheres are shown to consist of layers of oriented molecules aligned in the same direction. As these spheres continue to grow in size as heating is continued, they come in contact with one another and gradually coalesce with each other to produce larger masses of aligned layers. As coalescence continues, domains of aligned molecules much larger than those of the original spheres are formed. These domains come together to form a bulk mesophase wherein the transition from one oriented domain to another sometimes occurs smoothly and continuously through gradually curving lamellae and sometimes through more sharply curving lamellae. The differences in orientation between the domains create a complex array of polarized light extinction contours in the bulk mesophase corresponding to various types of linear discontinuity in molecular alignment. The ultimate size of the oriented domains produced is dependent upon the viscosity, and the rate of increase of the viscosity, of the mesophase from which they are formed, which, in turn are dependent upon the particular pitch and the heating rate. In certain pitches, domains having sizes in excess of two hundred microns and as large as several thousand microns are produced. In other pitches, the viscosity of the mesophase is such that only limited coalescence and structural rearrangement of layers occur, so that the ultimate domain size does not exceed one hundred microns.

The highly oriented, optically anisotropic, insoluble material produced by treating pitches in this manner has been given the term "mesophase", and pitches containing such material are known as "mesophase pitches". Such pitches, when heated above their softening points, are mixtures of two immiscible liquids, one the optically anisotropic, oriented mesophase portion, and the other the isotropic non-mesophase portion. The term "mesophase" is derived from the Greek "mesos" or "intermediate" and indicates the pseudo-crystalline nature of this highly-oriented, optically anisotropic material.

Carbonaceous pitches having a mesophase content of from about 40 per cent by weight to about 90 per cent by weight are suitable for producing the highly-oriented carbonaceous fibers capable of being thermoset to produce the highly-flexible, handleable fibers of the present invention. In order to obtain the desired fibers from such pitch, however, the mesophase contained therein must, under quiescent conditions, form a homogeneous bulk mesophase having large coalesced domains, i.e., domains of aligned molecules in excess of two hundred microns. Pitches which form stringy bulk mesophase under quiescent conditions, having small oriented domains, rather than large coalesced domains, are unsuitable. Such pitches form mesophase having a high viscosity which undergoes only limited coalescence, insufficient to produce large coalesced domains having sizes in excess of two hundred microns. Instead, small oriented domains of mesophase agglomerate to produce clumps or stringy masses wherein the ultimate domain size does not exceed one hundred microns. Certain pitches which polymerize very rapidly are of this type. Likewise, pitches which do not form a homogeneous bulk mesophase are unsuitable. The latter phenomenon is caused by the presence of infusible solids (which are either present in the original pitch or which develop on heating) which are enveloped by the coalescing mesophase and serve to interrupt the homogeneity and uniformity of the coalesced domains, and the boundaries between them.

Another requirement is that the pitch be nonthixotropic under the conditions employed in the spinning of the pitch into fibers, i.e., it must exhibit a Newtonian or plastic flow behavior so that the flow is uniform and well behaved. When such pitches are heated to a temperature where they exhibit a viscosity of from about 10 poises to about 200 poises, uniform fibers may be readily spun therefrom. Pitches, on the other hand, which do not exhibit Newtonian or plastic flow behavior at the temperature of spinning, do not permit uniform fibers to be spun therefrom.

Carbonaceous pitches having a mesophase content of from about 40 per cent by weight to about 90 per cent by weight can be produced in accordance with known techniques, as aforesaid, by heating a natural or synthetic carbonaceous pitch having an aromatic base in an inert atmosphere at a temperature above about 350° C. for a time sufficient to produce the desired quantity of mesophase. By an inert atmosphere is meant an atmosphere which does not react with the pitch under the heating conditions employed, such as nitrogen, argon, xenon, helium, and the like. The heating period required to produce the desired mesophase content varies with the particular pitch and temperature employed, with longer heating periods required at lower temperatures than at higher temperatures. At 350° C., the minimum temperature generally required to produce mesophase, at least one week of heating is usually necessary to

produce a mesophase content of about 40 per cent. At temperatures of from about 400° C. to 450° C., conversion to mesophase proceeds more rapidly, and a 50 per cent mesophase content can usually be produced at such temperatures within about 1-40 hours. Such temperatures are preferred for this reason. Temperatures above about 500° C. are undesirable, and heating at this temperature should not be employed for more than about 5 minutes to avoid conversion of the pitch to coke.

The degree to which the pitch has been converted to mesophase can readily be determined by polarized light microscopy and solubility examinations. Except for certain non-mesophase insolubles present in the original pitch or which, in some instances, develop on heating, the non-mesophase portion of the pitch is readily soluble in organic solvents such as quinoline and pyridine, while the mesophase portion is essentially insoluble. (1) In the case of pitches which do not develop non-mesophase insolubles when heated, the insoluble content of the heat-treated pitch over and above the insoluble content of the pitch before it has been heat-treated corresponds essentially to the mesophase content. (2) In the case of pitches which do develop non-mesophase insolubles when heated, the insoluble content of the heat-treated pitch over and above the insoluble content of the pitch before it has been heat treated is not solely due to the conversion of the pitch to mesophase, but also represents non-mesophase insolubles which are produced along with the mesophase during the heat treatment. Pitches which contain infusible non-mesophase insolubles (either present in the original pitch or developed by heating) in amounts sufficient to prevent the development of homogeneous bulk mesophase are unsuitable for producing highly-oriented carbonaceous fibers useful in the present invention, as noted above. Generally, pitches which contain in excess of about 2 per cent by weight of such infusible materials are unsuitable. The presence or absence of such homogeneous bulk mesophase regions, as well as the presence or absence of infusible non-mesophase insolubles, can be visually observed by polarized light microscopy examination of the pitch (see, e.g., Brooks, J. D., and Taylor, G. H., "The Formation of Some Graphitizing Carbons," *Chemistry and Physics of Carbon*, Vol. 4, Marcel Dekker, Inc., New York, 1968, pp. 243-268; and Dubois, J., Agache, C., and White, J. L., "The Carbonaceous Mesophase Formed in the Pyrolysis of Graphitizable Organic Materials," *Metallography* 3, pp. 337-269, 1970). The amounts of each of these materials may also be visually estimated in this manner.

(1) The percent of quinoline insolubles (Q.I.) of a given pitch is determined by quinoline extraction at 75° C. The per cent of pyridine insolubles (P.I.) is determined by Soxhlet extraction is boiling pyridine (115° C.).

(2) The insoluble content of the untreated pitch is generally less than 1 per cent (except for certain coal tar pitches) and consists largely of coke and carbon black found in the original pitch.

Aromatic base carbonaceous pitches having a carbon content of from about 92 per cent by weight to about 96 per cent by weight and a hydrogen content of from about 4 per cent by weight to about 8 per cent by weight are generally suitable for producing mesophase pitches which can be employed to produce the fibers useful in the instant invention. Elements other than carbon and hydrogen, such as oxygen, sulfur and nitrogen, are undesirable and should not be present in excess of about 4 per cent by weight. When such extraneous elements are present in amounts of from about 0.5 per cent by weight to about 4 per cent by weight, the

pitches generally have a carbon content of from about 92-95 per cent by weight, the balance being hydrogen.

Petroleum pitch, coal tar pitch and acenaphthylene pitch are preferred starting materials for producing the mesophase pitches which are employed to produce the fibers useful in the instant invention. Petroleum pitch can be derived from the thermal or catalytic cracking of petroleum fractions. Coal tar pitch is similarly obtained by the destructive distillation of coal. Both of these materials are commercially available natural pitches in which mesophase can easily be produced, and are preferred for this reason. Acenaphthylene pitch, on the other hand, is a synthetic pitch which is preferred because of its ability to produce excellent fibers. Acenaphthylene pitch can be produced by the pyrolysis of polymers of acenaphthylene as described by Edstrom et al, in U.S. Pat. No. 3,574,653.

Some pitches, such as fluoranthene pitch, polymerize very rapidly when heated and fail to develop large coalesced domains of mesophase, and are, therefore, not suitable precursor materials. Likewise, pitches having a high infusible non-mesophase insoluble content in organic solvents such as quinoline or pyridine, or those which develop a high infusible non-mesophase insoluble content when heated, should not be employed as starting materials, as explained above, because these pitches are incapable of developing the homogeneous bulk mesophase necessary to produce highly-oriented carbonaceous fibers. For this reason, pitches having an infusible quinoline-insoluble or pyridine-insoluble content of more than about 2 per cent by weight (determined as described above) should not be employed, or should be filtered to remove this material before being heated to produce mesophase. Preferably, such pitches are filtered when they contain more than about 1 per cent by weight of such infusible, insoluble material. Most petroleum pitches and synthetic pitches have a low infusible, insoluble content and can be used directly without such filtration. Most coal tar pitches, on the other hand, have a high infusible, insoluble content and require filtration before they can be employed.

As the pitch is heated at a temperature between 350° C. and 500° C. to produce mesophase, the pitch will, of course, pyrolyze to a certain extent and the composition of the pitch will be altered, depending upon the temperature, the heating time, and the composition and structure of the starting material. Generally, however, after heating a carbonaceous pitch for a time sufficient to produce a mesophase content of from about 40 per cent by weight to about 90 per cent by weight, the resulting pitch will contain a carbon content of from about 94-96 per cent by weight and a hydrogen content of from about 4-6 per cent by weight. When such pitches contain elements other than carbon and hydrogen in amounts of from about 0.5 per cent by weight to about 4 per cent by weight, the mesophase pitch will generally have a carbon content of from about 92-95 per cent by weight, the balance being hydrogen.

After the desired mesophase pitch has been prepared, it is spun into fiber by conventional techniques, e.g., by melt spinning, centrifugal spinning, blow spinning, or in any other known manner. As noted above, in order to obtain highly-oriented carbonaceous fibers capable of being thermoset to produce the highly-flexible, handleable fibers of the present invention, the pitch must, under quiescent conditions, form a homogeneous bulk mesophase having large coalesced domains, and be nonthixotropic under the conditions employed in the

spinning. Further, in order to obtain uniform fibers from such pitch, the pitch should be agitated immediately prior to spinning so as to effectively intermix the immiscible mesophase and non-mesophase portions of the pitch.

The temperature at which the pitch is spun depends, of course, upon the temperature at which the pitch exhibits a suitable viscosity, and at which the higher-melting mesophase portion of the pitch can be easily deformed and oriented. Since the softening temperature of the pitch, and its viscosity at a given temperature, increases as the mesophase content of the pitch increases, the mesophase content should not be permitted to rise to a point which raises the softening point of the pitch to excessive levels. For this reason, pitches having a mesophase content of more than about 90 per cent are generally not employed. Pitches containing a mesophase content of from about 40 per cent by weight to about 90 per cent by weight, however, generally exhibit a viscosity of from about 10 poises to about 200 poises at temperatures of from about 310° C. to above about 450° C. and can be readily spun at such temperatures. Preferably, the pitch employed has a mesophase content of from about 45 per cent by weight to about 75 per cent by weight, most preferably from about 55 per cent by weight to about 75 per cent by weight, and exhibits a viscosity of from about 30 poises to about 150 poises at temperatures of from about 340° C. to about 440° C. At such viscosity and temperature, uniform fibers having diameters of from about 6 microns to about 14 microns can be easily spun. Such small diameter fibers are preferred because of their increased handleability. As previously mentioned, however, in order to obtain the desired fibers, it is important that the pitch be nonthixotropic and exhibit Newtonian or plastic flow behavior during the spinning of the fibers.

After the carbonaceous fibers have been spun, they are oxidized to an oxygen content of from 17 per cent by weight to 30 per cent by weight, preferably from 18 per cent by weight to 22 per cent by weight, by heating in an oxygen atmosphere. The oxygen atmosphere employed may be pure oxygen, nitric oxide, or any other appropriate oxidizing atmosphere. Most conveniently, air is employed as the oxidizing atmosphere.

The time required to oxidize the fibers to the desired degree will, of course, vary with such factors as the particular oxidizing atmosphere, the temperature employed, the diameter of the fibers, the particular pitch from which the fibers are prepared, and the mesophase content of such pitch. Generally, however, in excess of 60 minutes heating are required to effect the desired degree of oxidation, usually from about 120 minutes to about 240 minutes.

The temperature at which the fibers are oxidized must, of course, not exceed the temperature at which the fibers will soften or distort. The maximum temperature which can be employed will thus depend upon the particular pitch from which the fibers were spun, and the mesophase content of such pitch. The higher the mesophase content of the fiber, the higher will be its softening temperature, and the higher the temperature which can be employed to effect oxidation. At higher temperatures, of course, oxidation can be effected in less time than is possible at lower temperatures. Fibers having a lower mesophase content, on the other hand, require relatively longer heat treatment at somewhat lower temperatures to effect the desired degree of oxidation.

A minimum temperature of at least 250° C. is generally necessary to effect oxidation of the fibers. Temperatures in excess of 500° C. may cause melting and/or excessive burn-off of the fibers and should be avoided. Preferably, temperatures of from about 275° C. to about 390° C. are employed.

The oxidized fibers produced in this manner have a high degree of flexibility and handleability, a strain-to-failure of at least 5 per cent, and a tensile strength of at least 30,000 psi., usually at least 35,000 psi. These properties enable continuous fiber lengths to be easily tied in a knot, processed at high speeds by means of conventional yarn-transport systems, and readily woven or knit into cloth. Such cloth may then be processed to carbon or graphite form by further heat treatment, thereby eliminating the difficulty of weaving or knitting cloth from fibers which have been stiffened to a high modulus by such thermal treatment. When staple length fibers are produced, they may be used to produce continuous length fibers by means of conventional techniques.

After the fibers have been oxidized to the extent necessary and, if desired, woven or knit into cloth, they are heated to a carbonizing temperature so as to expel hydrogen and other volatiles. At a temperature of about 1000° C., fibers having a carbon content greater than about 98 per cent by weight are obtained. At temperatures in excess of 1500° C., the fibers are substantially completely carbonized. Such heating should be conducted in an oxygen-free atmosphere, such as the inert atmospheres described above, to prevent further oxidation of the fibers.

Usually, carbonization is effected at a temperature of from about 1000° C. to about 2500° C., preferably from about 1400° C. to about 1700° C. Generally, residence times of no more than about 60 minutes are employed. While more extended heating times can be employed with good results, such residence times are uneconomical and, as a practical matter, there is no advantage in employing such long periods. In order to ensure that the rate of weight loss of the fibers does not become so excessive as to disrupt the fiber structure, it is preferred to gradually heat the fibers to their final carbonization temperature.

If desired, the carbonized fibers may be further heated in an inert atmosphere, as described hereinbefore, to a graphitizing temperature in a range of from

understand the invention. It should be understood that it is exemplary only, and should not be construed as limiting the invention in any manner. Tensile strengths referred to in the examples and throughout the specification, unless otherwise indicated, were measured on 10 cm. length unidirectional fiber-epoxy composites. Young's modulus was measured on 2.0 cm. lengths of individual filaments unless otherwise indicated.

#### EXAMPLE 1

A commercial petroleum pitch was employed to produce a pitch having a mesophase content of about 56 per cent by weight. The precursor pitch had a density of 1.23 Mg./m.<sup>3</sup>, a softening temperature of 120° C. and contained 0.3 per cent by weight quinoline insolubles (Q.I. was determined by quinoline extraction at 75° C.).

The mesophase pitch was produced by heating the precursor petroleum pitch at a temperature of about 400° C. for about 19 hours under flowing nitrogen. The pitch was continuously stirred during this time and nitrogen gas was continuously bubbled through the pitch. After heating, the pitch exhibited a softening point of 341° C. and contained 56.6 per cent by weight pyridine insolubles, indicating that the pitch had a mesophase content of close to 56 per cent.

A portion of the pitch produced in this manner was then melt spun into fibers at a rate of 325 meters per minute through a 240 hole spinnerette (0.07 mm. diameter holes) at a temperature of 385° C. The filaments passed through a nitrogen atmosphere as they left the spinnerette and were then taken up by a reel. A considerable quantity of fiber 9-12 microns in diameter was produced in this manner.

A portion of the spun filaments were placed in a stainless steel wire mesh tray and heated in a forced-air convection oven to a temperature of 315° C. over a period of 45 minutes. This procedure was repeated a number of times with different portions of the spun filaments, except that varying hold times at 315° C. were employed with each successive portion so as to vary the exposure time of each portion to the oxidizing atmosphere and the resulting oxygen content of the fibers of each lot. The oxygen content, tensile strength and modulus of the fibers produced in each run was then determined. The results of these experiments are set forth in Table I below:

Table I

Mechanical Properties of Thermoset Mesophase Pitch Fibers as a Function of Oxygen Content

| Run No. | Hold Time at 315° C., Min. | Composition, % | Tensile Strength, kpsi. | Young's Modulus, Mpsi. | Strain to Failure, % |
|---------|----------------------------|----------------|-------------------------|------------------------|----------------------|
|         |                            | 0 C H          |                         |                        |                      |
| 1       | 0                          | 8.5 89.4 3.3   | —                       | 0.65                   | —                    |
| 2       | 15                         | 13.3 85.0 3.0  | 17                      | 0.80                   | 2.1                  |
| 3       | 30                         | 14.8 83.3 2.7  | 20                      | 0.71                   | 2.8                  |
| 4       | 45                         | 15.4 81.2 2.6  | 21                      | 0.66                   | 3.2                  |
| 5       | 60                         | 16.2 80.2 2.6  | 27                      | 0.52                   | 5.2                  |
| 6       | 90                         | 17.4 79.4 2.5  | 31                      | 0.66                   | 4.7                  |
| 7       | 180                        | 18.7 78.3 2.2  | 37                      | 0.63                   | 5.6                  |
| 8       | 240                        | 20.3 77.3 2.2  | 36                      | 0.72                   | 5.0                  |
| 9       | 1160                       | 26.3 71.1 1.8  | 33                      | —                      | —                    |

above about 2500° C. to about 3300° C., preferably from about 2800° C. to about 3000° C. A residence time of about 1 minute is satisfactory, although both shorter and longer times may be employed, e.g., from about 1 second to about 5 minutes, or longer. Residence times longer than 5 minutes are uneconomical and unnecessary, but may be employed if desired.

The following example is set forth for purposes of illustration so that those skilled in the art may better

60  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
550  
551  
552  
553  
554  
555  
556  
557  
558  
559  
560  
561  
562  
563  
564  
565  
566  
567  
568  
569  
560  
561  
562  
563  
564  
565  
566  
567  
568  
569  
570  
571  
572  
573  
574  
575  
576  
577  
578  
579  
580  
581  
582  
583  
584  
585  
586  
587  
588  
589  
580  
581  
582  
583  
584  
585  
586  
587  
588  
589  
590  
591  
592  
593  
594  
595  
596  
597  
598  
599  
590  
591  
592  
593  
594  
595  
596  
597  
598  
599  
600  
601  
602  
603  
604  
605  
606  
607  
608  
609  
600  
601  
602  
603  
604  
605  
606  
607  
608  
609  
610  
611  
612  
613  
614  
615  
616  
617  
618  
619  
610  
611  
612  
613  
614  
615  
616  
617  
618  
619  
620  
621  
622  
623  
624  
625  
626  
627  
628  
629  
620  
621  
622  
623  
624  
625  
626  
627  
628  
629  
630  
631  
632  
633  
634  
635  
636  
637  
638  
639  
630  
631  
632  
633  
634  
635  
636  
637  
638  
639  
640  
641  
642  
643  
644  
645  
646  
647  
648  
649  
640  
641  
642  
643  
644  
645  
646  
647  
648  
649  
650  
651  
652  
653  
654  
655  
656  
657  
658  
659  
650  
651  
652  
653  
654  
655  
656  
657  
658  
659  
660  
661  
662  
663  
664  
665  
666  
667  
668  
669  
660  
661  
662  
663  
664  
665  
666  
667  
668  
669  
670  
671  
672  
673  
674  
675  
676  
677  
678  
679  
670  
671  
672  
673  
674  
675  
676  
677  
678  
679  
680  
681  
682  
683  
684  
685  
686  
687  
688  
689  
680  
681  
682  
683  
684  
685  
686  
687  
688  
689  
690  
691  
692  
693  
694  
695  
696  
697  
698  
699  
690  
691  
692  
693  
694  
695  
696  
697  
698  
699  
700  
701  
702  
703  
704  
705  
706  
707  
708  
709  
700  
701  
702  
703  
704  
705  
706  
707  
708  
709  
710  
711  
712  
713  
714  
715  
716  
717  
718  
719  
710  
711  
712  
713  
714  
715  
716  
717  
718  
719  
720  
721  
722  
723  
724  
725  
726  
727  
728  
729  
720  
721  
722  
723  
724  
725  
726  
727  
728  
729  
730  
731  
732  
733  
734  
735  
736  
737  
738  
739  
730  
731  
732  
733  
734  
735  
736  
737  
738  
739  
740  
741  
742  
743  
744  
745  
746  
747  
748  
749  
740  
741  
742  
743  
744  
745  
746  
747  
748  
749  
750  
751  
752  
753  
754  
755  
756  
757  
758  
759  
750  
751  
752  
753  
754  
755  
756  
757  
758  
759  
760  
761  
762  
763  
764  
765  
766  
767  
768  
769  
760  
761  
762  
763  
764  
765  
766  
767  
768  
769  
770  
771  
772  
773  
774  
775  
776  
777  
778  
779  
770  
771  
772  
773  
774  
775  
776  
777  
778  
779  
780  
781  
782  
783  
784  
785  
786  
787  
788  
789  
780  
781  
782  
783  
784  
785  
786  
787  
788  
789  
790  
791  
792  
793  
794  
795  
796  
797  
798  
799  
790  
791  
792  
793  
794  
795  
796  
797  
798  
799  
800  
801  
802  
803  
804  
805  
806  
807  
808  
809  
800  
801  
802  
803  
804  
805  
806  
807  
808  
809  
810  
811  
812  
813  
814  
815  
816  
817  
818  
819  
810  
811  
812  
813  
814  
815  
816  
817  
818  
819  
820  
821  
822  
823  
824  
825  
826  
827  
828  
829  
820  
821  
822  
823  
824  
825  
826  
827  
828  
829  
830  
831  
832  
833  
834  
835  
836  
837  
838  
839  
830  
831  
832  
833  
834  
835  
836  
837  
838  
839  
840  
841  
842  
843  
844  
845  
846  
847  
848  
849  
840  
841  
842  
843  
844  
845  
846  
847  
848  
849  
850  
851  
852  
853  
854  
855  
856  
857  
858  
859  
850  
851  
852  
853  
854  
855  
856  
857  
858  
859  
860  
861  
862  
863  
864  
865  
866  
867  
868  
869  
860  
861  
862  
863  
864  
865  
866  
867  
868  
869  
870  
871  
872  
873  
874  
875  
876  
877  
878  
879  
870  
871  
872  
873  
874  
875  
876  
877  
878  
879  
880  
881  
882  
883  
884  
885  
886  
887  
888  
889  
880  
881  
882  
883  
884  
885  
886  
887  
888  
889  
890  
891  
892  
893  
894  
895  
896  
897  
898  
899  
890  
891  
892  
893  
894  
895  
896  
897  
898  
899  
900  
901  
902  
903  
904  
905  
906  
907  
908  
909  
900  
901  
902  
903  
904  
905  
906  
907  
908  
909  
910  
911  
912  
913  
914  
915  
916  
917  
918  
919  
910  
911  
912  
913  
914  
915  
916  
917  
918  
919  
920  
921  
922  
923  
924  
925  
926  
927  
928  
929  
920  
921  
922  
923  
924  
925  
926  
927  
928  
929  
930  
931  
932  
933  
934  
935  
936  
937  
938  
939  
930  
931  
932  
933  
934  
935  
936  
937  
938  
939  
940  
941  
942  
943  
944  
945  
946  
947  
948  
949  
940  
941  
942  
943  
944  
945  
946  
947  
948  
949  
950  
951  
952  
953  
954  
955  
956  
957  
958  
959  
950  
951  
952  
953  
954  
955  
956  
957  
958  
959  
960  
961  
962  
963  
964  
965  
966  
967  
968  
969  
960  
961  
962  
963  
964  
965  
966  
967  
968  
969  
970  
971  
972  
973  
974  
975  
976  
977  
978  
979  
970  
971  
972  
973  
974  
975  
976  
977  
978  
979  
980  
981  
982  
983  
984  
985  
986  
987  
988  
989  
980  
981  
982  
983  
984  
985  
986  
987  
988  
989  
990  
991  
992  
993  
994  
995  
996  
997  
998  
999  
990  
991  
992  
993  
994  
995  
996  
997  
998  
999  
1000  
1001  
1002  
1003  
1004  
1005  
1006  
1007  
1008  
1009  
1000  
1001  
1002  
1003  
1004  
1005  
1006  
1007  
1008  
1009  
1010  
1011  
1012  
1013  
1014  
1015  
1016  
1017  
1018  
1019  
1010  
1011  
1012  
1013  
1014  
1015  
1016  
1017  
1018  
1019  
1020  
1021  
1022  
1023  
1024  
1025  
1026  
1027  
1028  
1029  
1020  
1021  
1022  
1023  
1024  
1025  
1026  
1027  
1028  
1029  
1030  
1031  
1032  
1033  
1034  
1035  
1036  
1037  
1038  
1039  
1030  
1031  
1032  
1033  
1034  
1035  
1036  
1037  
1038  
1039  
1040  
1041  
1042  
1043  
1044  
1045  
1046  
1047  
1048  
1049  
1040  
1041  
1042  
1043  
1044  
1045  
1046  
1047  
1048  
1049  
1050  
1051  
1052  
1053  
1054  
1055  
1056  
1057  
1058  
1059  
1050  
1051  
1052  
1053  
1054  
1055  
1056  
1057  
1058  
1059  
1060  
1061  
1062  
1063  
1064  
1065  
1066  
1067  
1068  
1069  
1060  
1061  
1062  
1063  
1064  
1065  
1066  
1067  
1068  
1069  
1070  
1071  
1072  
1073  
1074  
1075  
1076  
1077  
1078  
1079  
1070  
1071  
1072  
1073  
1074  
1075  
1076  
1077  
1078  
1079  
1080  
1081  
1082  
1083  
1084  
1085  
1086  
1087  
1088  
1089  
1080  
1081  
1082  
1083  
1084  
1085  
1086  
1087  
1088  
1089  
1090  
1091  
1092  
1093  
1094  
1095  
1096  
1097  
1098  
1099  
1090  
1091  
1092  
1093  
1094  
1095  
1096  
1097  
1098  
1099  
1100  
1101  
1102  
1103  
1104  
1105  
1106  
1107  
1108  
1109  
1100  
1101  
1102  
1103  
1104  
1105  
1106  
1107  
1108  
1109  
1110  
1111  
1112  
1113  
1114  
1115  
1116  
1117  
1118  
1119  
1110  
1111  
1112  
1113  
1114  
1115  
1116  
1117  
1118  
1119  
1120  
1121  
1122  
1123  
1124  
1125  
1126  
1127  
1128  
1129  
1120  
1121  
1122  
1123  
1124  
1125  
1126  
1127  
1128  
1129  
1130  
1131  
1132  
1133  
1134  
1135  
1136  
1137  
1138  
1139  
1130  
1131  
1132  
1133  
1134  
1135  
1136  
1137  
1138  
1139  
1140  
1141  
1142  
1143  
1144  
1145  
1146  
1147  
1148  
1149  
1140  
1141  
1142  
1143  
11

spinning a carbonaceous fiber from a nonthixotropic carbonaceous pitch having a mesophase content of from 40 per cent by weight to 90 per cent by weight which under quiescent conditions forms a homogeneous bulk mesophase having large coalesced domains; and heating the spun fiber in an oxygen-containing atmosphere at a temperature of from 250° C. to 500° C. for a time sufficient to oxidize the fiber to an oxygen content of from 17 per cent by weight to 30 per cent by weight to produce a fiber having a tensile strength of at least 30,000 psi. and a strain-to-failure of at least 5 per cent.

2. A process as in claim 1 wherein the carbonaceous fiber which is spun from the carbonaceous pitch has a diameter of from 6 microns to 14 microns.

3. A process as in claim 1 wherein the spun fiber is oxidized to an oxygen content of from 18 per cent by weight to 22 per cent by weight.

4. A process as in claim 3 wherein the carbonaceous fiber which is spun from the carbonaceous pitch has a diameter of from 6 microns to 14 microns.

5. A process as in claim 1 wherein the oxygen-containing atmosphere is air and the spun fiber is heated in said atmosphere at a temperature of from 275° C. to 390° C.

6. A process as in claim 5 wherein the carbonaceous fiber which is spun from the carbonaceous pitch has a diameter of from 6 microns to 14 microns.

7. A process as in claim 5 wherein the spun fiber is oxidized to an oxygen content of from 18 per cent by weight to 22 per cent by weight.

8. A process as in claim 7 wherein the carbonaceous fiber which is spun from the carbonaceous pitch has a diameter of from 6 microns to 14 microns.

9. In a process for producing carbon fiber which comprises spinning a carbonaceous fiber from a non-thixotropic carbonaceous pitch having a mesophase content of from 40 per cent by weight to 90 per cent by weight which under quiescent conditions forms a homogeneous bulk mesophase having large coalesced domains; heating the spun fiber in an oxygen-containing atmosphere at a temperature of from 250° C. to 500° C. for a time sufficient to render it infusible; and carbonizing the infusible fiber so produced by heating in an inert atmosphere; the improvement which comprises oxidizing the spun fiber to an oxygen content of from 17 per cent by weight to 30 per cent by weight to produce a

fiber having a tensile strength of at least 30,000 psi. and a strain-to-failure of at least 5 per cent.

10. A process as in claim 9 wherein the carbonaceous fiber which is spun from the carbonaceous pitch has a diameter of from 6 microns to 14 microns.

11. A process as in claim 9 wherein the spun fiber is oxidized to an oxygen content of from 18 per cent by weight to 22 per cent by weight.

12. A process as in claim 11 wherein the carbonaceous fiber which is spun from the carbonaceous pitch has a diameter of from 6 microns to 14 microns.

13. A process as in claim 9 wherein the oxygen-containing atmosphere is air and the spun fiber is heated in said atmosphere to a temperature of from 275° C. to 390° C.

14. A process as in claim 13 wherein the carbonaceous fiber which is spun from the carbonaceous pitch has a diameter of from 6 microns to 14 microns.

15. A process as in claim 13 wherein the spun fiber is oxidized to an oxygen content of from 18 per cent by weight to 22 per cent by weight.

16. A process as in claim 15 wherein the carbonaceous fiber which is spun from the carbonaceous pitch has a diameter of from 6 microns to 14 microns.

17. Carbonaceous fiber prepared by oxidizing a pitch fiber having a mesophase content of from 40 per cent by weight to 90 per cent by weight to an oxygen content of from 17 per cent by weight to 30 per cent by weight, said fiber having a tensile strength of at least 30,000 psi. and a strain-to-failure of at least 5 per cent.

18. A fiber as in claim 17 having a diameter of from 6 microns to 14 microns.

19. A fiber as in claim 17 having an oxygen content of from 18 per cent by weight to 22 per cent by weight.

20. A fiber as in claim 19 having a diameter of from 6 microns to 14 microns.

21. A fiber as in claim 17 having a tensile strength of at least 35,000 psi.

22. A fiber as in claim 21 having a diameter of from 6 microns to 14 microns.

23. A fiber as in claim 21 having an oxygen content of from 18 per cent by weight to 22 per cent by weight.

24. A fiber as in claim 23 having a diameter of from 6 microns to 14 microns.

\* \* \* \* \*

UNITED STATES PATENT OFFICE  
CERTIFICATE OF CORRECTION

Patent No. 4,138,525

Dated February 6, 1979

Inventor(s) David A. Schulz

It is certified that error appears in the above-identified patent and that said Letters Patent are hereby corrected as shown below:

Column 4, line 5, the comma (,) after "hours" should be a period (.).

Column 4, line 14, "deveop" should read -- develop --.

Column 4, line 49, "337-269" should read -- 337-369 --.

Column 5, line 16, the comma (,) after "al" should be a period (.).

Signed and Sealed this

*Nineteenth Day of June 1979*

[SEAL]

Attest:

RUTH C. MASON  
*Attesting Officer*

DONALD W. BANNER  
*Commissioner of Patents and Trademarks*